

Patented May 22, 1928.

1,671,034

# UNITED STATES PATENT OFFICE.

ANDREAS LENNARTZ, OF NEAR AACHEN, GERMANY.

## CASE HARDENING.

No Drawing. Application filed January 25, 1927, Serial No. 163,559, and in Germany February 15, 1926.

In case-hardening articles of iron or iron alloys there is often desired only a partial surface-hardening. To this end, the portions to be kept soft are covered during the cementation process with a suitable protective mass. However, the protective masses such as kaolin, loam, et cetera used hitherto do not give surety for completely preventing the diffusion of carbon into the portions not 10 to be hardened during the cementation.

The invention has for its object to avoid the said drawback by adding a sulphide, for instance ferrous sulphide, to the known protective masses. It has been proved by 15 numerous tests that a sulphide added to the said protective masses securely prevents during the cementation process any penetration of carbon into those portions of the articles treated which are designed to remain un- 20 hardened.

Having thus described my invention, what I claim as new and desire to secure by Letters-Patent is:—

1. An improved composition of matter used in selective case-hardening, including 25 the addition of ferrous-sulphide to the composition employed to protect portions of the article being case-hardened against such action.

2. An improved composition of matter 30 used in selective case-hardening, including the addition of a sulphide to the composition employed to protect portions of the article being case-hardened against such action.

In testimony whereof I have signed my 35 name to this specification.

ANDREAS LENNARTZ.